

W. H. SAUNDERS.

Axle-Box.

No. 16,153.

Patented Dec. 2, 1856.

Fig. 3.



Fig. 5.



Fig. 2.



Fig. 4.



Fig. 1.



# UNITED STATES PATENT OFFICE.

WM. H. SAUNDERS, OF HASTINGS-UPON-HUDSON, NEW YORK.

## AXLE-BOX.

Specification of Letters Patent No. 16,153, dated December 2, 1856.

*To all whom it may concern:*

Be it known that I, WM. H. SAUNDERS, of Hastings-upon-Hudson, Westchester county, New York, have invented certain new and 5 useful Improvements in Boxes for Axles, and that the following specification, taken in connection with the drawings, is a full, clear, and exact description thereof.

In the drawings Figure 1 is an end view 10 of my box from the side nearest the vehicle. Fig. 2 is an elevation thereof. Fig. 3 is an end view of the box at the smaller end thereof. Fig. 4 is a longitudinal section through the box and Fig. 5 is a cross section on the line X X of Fig. 2.

My invention relates to cylindrical axles of all sorts for vehicles and is intended to obviate certain difficulties, which arise when they are used as at present constructed, 20 while the expense of construction is not materially increased.

The requisites of a good cylindrical box are first that it should be truly cylindrical so as to avoid play and consequent rattling 25 when the axle slips endwise in the box, from wear, or compression of the washers. Second that the material should be highly polished, so as to diminish friction as much as possible. Third that the metal should be 30 hard so as not to cut away readily nor to lose its shape when subjected to violent concussions of the axle against the interior of the box; and fourth the box if possible should be made of a metal that expands by 35 heat in a greater ratio than the axle itself so that there should be no sticking when the axle arm heats up.

The ordinary cast iron axle box fulfills 40 the three first requisitions—it is susceptible of being truly bored out, highly polished, and is of sufficient hardness, but cast iron is as may be seen by reference to tables of dilation of different bodies by heat, less increased in bulk by equal increments of heat 45 than wrought iron. Hence it follows that when an axle heats, it usually sticks in the box, and either wrings open the hub or twists itself off at its collar. It has been attempted to obviate this latter difficulty 50 by making the whole box of cast brass, or by lining it with Babbitt metal cast into it; but a brass box is too expensive and is not sufficiently hard while the Babbitt metal lining is not only much too soft to stand the 55 concussion, but also melts out when the axle becomes heated. When it melts, the

axle arm cuts itself to pieces on the irregular shaped iron box. Now it has occurred to me that by lining the box with a condensed thin drawn tube of copper or some compound thereof such as brass or German silver or with metals or compounds having similar qualities in regard to dilation as compared with iron and capable of being hardened by condensation that I could secure all the advantages required in a higher degree than usual; could obviate the difficulty of sticking when heated, or at any rate the danger incident thereto, and further could furnish a box having less friction 70 than those now in use. These advantages can moreover be attained at a moderate increase of cost.

The nature of my invention therefore consists in lining an axle box substantially 75 in the manner hereinafter described with a thin tube of condensed and therefore hardened copper or some of the alloys thereof such as German silver or brass or with a thin tube similarly hardened of some metal 80 or alloys capable of being condensed and so affected by heat as to increase in bulk in a greater ratio than wrought iron.

In order to carry out my invention I take 85 a tube of brass, German silver or similar substance either brazed or seamless, but best made of sheet metal hardened by rolling and brazed, and draw it down over a polished steel mandrel of the same diameter as the box and through dies gradually decreasing in size, until the metal begins to tear and break or until sufficiently hardened. I prefer to make the last die or the last two 90 or three dies polygonal or fluted so as to give a corresponding shape to the exterior 95 of the tube. When this tube is cut up into proper lengths it is shoved into a cast iron box properly bored and chlorid of zinc, is introduced between the tube and box. The whole is then subjected to heat until the two 100 surfaces are soldered to each other. Other methods of securing the tube in the box may be used, and the ends of the tube may be expanded or swelled over the ends of the cylinder in which it rests, so as to prevent 105 its slipping endwise even if the solder should melt. By such means I procure a tube with a hard polished interior surface so thin that the box as a whole is not enlarged in diameter and at no great increase 110 of cost over a common box. This tube moreover expands faster than the axle

which it contains and when heated will tend to free itself compressing the solder. When much heated all that can happen is that the solder should melt out and then the box will 5 revolve around the lining; there can be no danger of splitting hubs or twisting off axles. Such a box will induce much less friction than one wholly composed of brass or copper as the latter cannot be hardened 10 and it will cost less. The pipe cannot melt out as is the case with a Babbitt metal lining and even if the solder melts the axle will not cut and a resoldering will make the whole as serviceable as ever.

15 In the drawings the iron of the box is shown at *a a*, the lining at *b b* while the expansion of the lining at one end is shown at *c c*.

Having thus described my improved axle box I claim therein as new and of my own 20 invention—

A lining of a thin tube of condensed and hardened ductile metal or composition substantially such as is herein specified, introduced and secured within the box and presenting a hard polished surface to the axle itself substantially in the manner and for the purposes described.

In testimony whereof I have hereunto subscribed my name in presence of two witnesses on this 2 day of Feby. A. D. 1856.

W. H. SAUNDERS.

Witnesses:

P. D. KELLY,  
JOHN MORRIS.